

## UNITED STATES PATENT OFFICE

WILHELM ECKERT, OF FRANKFORT-ON-THE-MAIN-HOCHST, AND WERNER KIRST, OF FRANKFORT-ON-THE-MAIN, GERMANY, ASSIGNORS TO GENERAL ANILINE WORKS, INC., OF NEW YORK, N. Y., A CORPORATION OF DELAWARE

## AZO DYESTUFFS AND MATERIAL DYED THEREWITH

No Drawing. Application filed December 3, 1928, Serial No. 323,555, and in Germany December 10, 1927.

The present invention relates to azo dye-stuffs and material dyed therewith. The free sulfonic or carboxylic group and Y stands for hydrogen or for the residue:

We have found that claret, violet and violet-brown azo dyestuffs are obtained by diazotizing a 4-amino-naphthalic acid derivative of the following constitution:



15 wherein X stands for hydrogen, alkyl, aryl or aralkyl and which may be substituted or not, and coupling the diazotized product in substance or on the fiber with 2,3-hydroxynaphthoic acid arylamide. These azo dye-stuffs yield tints, which are distinguished by a good to excellent fastness to light.

20 The new dyestuffs correspond to the general formula:



40 wherein X stands for hydrogen, alkyl, aryl or aralkyl and wherein the aryl residue may 45 be substituted or not, but must contain no



wherein X has the same meaning as in the preceding formula.

The 4-aminonaphthalic acid derivatives may for instance be prepared from the 4-aminonaphthalic anhydride or a substitution product thereof by decomposing it with ammonia, with an aliphatic or aromatic amine.

The following examples serve to illustrate our invention, but they are not intended to limit it thereto.

1. (a) 50 grammes of boiled cotton yarn are treated for about  $\frac{1}{2}$  hour with the following grounding liquor: 4.5 grammes of 2,3-hydroxynaphthoic acid-2'-5'-dimethoxy-1'-anilide, 9 ccm. of Turkey red oil and 9 cc. of caustic soda solution of 34° Bé. are dissolved while boiling in hot water and the whole is made up to 1000 cc. Then 4.5 cc. of formaldehyde of 30% strength are added.

(b) The impregnated yarn is well freed from water and developed in a diazo solution prepared in the following manner:

2.2 grammes of 4-amino-1,8-naphthalimide are made into a paste with 2.8

75

80

cc. of hydrochloric acid of 22° Bé. and 3 cc. of hot water and diazotized by means of 7.5 cc. of sodium nitrite dissolved in water in the proportion of 1:10.

5 The diazotization being completed, the whole is neutralized with about 2 grammes of sodium acetate, dissolved in water, so as to indicate neutral reaction towards Congo paper, 25 grammes of sodium chloride are added and the liquor is made up with cold spring water to 1 liter.

10 After about 1/2 hour's dyeing, the yarn is taken out, well mixed, soaped at boiling temperature, again rinsed and dried.

15 A beautiful, very bluish claret dyeing is obtained of excellent fastness to light. The dyestuff has the following formula:



2: 50 grammes of boiled cotton yarn are 35 treated with the following grounding liquor: 4 grammes of 2,3-hydroxynaphthoic acid 1'-naphthylamide, 8 cc. of Turkey red oil, 12 cc. of caustic soda solution of 34° Bé. are dissolved while boiling in hot water and the whole is made up to 1000 cc. Then there 40 are added 4 cc. of formaldehyde of 30% strength.

The whole is developed with a diazo solution from 4-amino-1,8-naphthalamide, the developed dyeing is treated as indicated in Example 1 and a beautiful, blue Bordeaux dyeing of very good fastness to light is obtained. The dyestuff has the following formula:



65 3. 50 grammes of boiled cotton yarn are

treated with the following grounding bath: 2 grammes of di-2,3-hydroxynaphthoic acid-dianisidine, 10 cc. of Turkey red oil of 50% strength and 6 cc. of caustic soda solution of 34° Bé. are dissolved in boiling water and the whole is made up to 1 liter.

70 The dyeing is developed with a diazo solution from 4-amino-1,8-naphthalamide and further treated as indicated in Example 1. A violet brown of very good fastness to light is obtained. The dyestuff has the following formula:



4. 50 grammes of boiled cotton yarn are treated in a solution prepared according to Example 1 from 4.5 grammes of 2,3-hydroxynaphthoic acid - 2',5' - dimethoxy-1 - anilide and dyed in the following bath:

95 2.06 grammes of 4-amino-1,8-naphthalamide are diazotized in the cold with 2.8 cc. of hydrochloric acid of 22° Bé. and 7.5 cc. of a solution of sodium nitrite in water containing 1 g. in 10 cc. After the diazotization is complete, the mass is neutralized with about 2 grammes of dissolved sodium acetate so that it gives a neutral reaction with Congo paper and the whole is made up with addition of 25 grammes of sodium chloride to 1 liter. After having developed for about 1/2 hour, the yarn is rinsed, soaped at boiling temperature and dried. A beautiful claret-red dyeing of excellent fastness to light is obtained. The dyestuff has the following formula:



130 5. 50 grammes of boiled cotton yarn are

treated with the following grounding liquor: 7 grammes of 2,3-hydroxynaphthoic acid anilide, 14 cc. of Turkey red oil of 50% strength and 10.5 cc. of caustic soda solution of 34° Bé. are dissolved in boiling water and the solution is made up to 1 liter. Then there are added 7 cc. of formaldehyde of 30% strength. After grounding for 1/2 hour, the yarn is dyed in a developing bath prepared as indicated in Example 4 from 4-amino-1,8-naphthalimide and treated as above indicated. A violet tint of good fastness to light is obtained. The dyestuff has the following formula:

15



20

25

solved in boiling water together with 9 cc. of Turkey red oil of 50% strength and 9 cc. of caustic soda solution of 34° Bé. and the whole is made up to 1 liter. Then there are added 4.5 cc. of formaldehyde of 30% strength. The naphtholated yarn is developed in a diazo solution prepared according to Example 4 from 4-amino-1,8-naphthalimide and after-treated in the above indicated manner. A violet tint of good to very good fastness to light is obtained. The dyestuff has the following formula:

60

65

70



6. 50 grammes of boiled cotton yarn are treated in a solution of 4 grammes of 2,3-hydroxynaphthoic acid - 1' - naphthyleamide (prepared according to Example 2 and developed with a diazo solution prepared according to Example 4). The material is soaped at boiling temperature, rinsed and dried. A violet tint of good fastness to light is obtained. The dyestuff has the following formula:

40

45

50



8. 50 grammes of boiled cotton yarn are treated with a grounding liquor prepared as indicated in Example 3 from 2-grammes of di - 2,3 - hydroxynaphthoic acid-dianiside. Then the dyeing is developed in a diazo solution prepared according to Example 4 from 4-amino-1,8-naphthalimide, rinsed, soaped at boiling temperature, dried and a chocolate brown tint of very good fastness to light is obtained. The dyestuff has the following formula:

85

90

95



7. 50 grammes of boiled cotton yarn are impregnated with the following naphthol solution: 4.5 grammes of 2,3-hydroxy-naphthoic acid-4'-methoxy-1'-anilide are dis-

The following table illustrates a number of the dyestuffs obtained according to the examples, but it is not to be understood as limiting the possibility to obtain similar dye-

stuffs of equally good fastness properties by some other combinations of the base and the coupling component, than those included in the table.

let or violet-brown dyestuffs of good fastness to washing and chlorine and good to excellent fastness to light.

2. As new products, azo dyestuffs of the 65

5

| Diazo compound from— |                                                                                                                                                                                                                                                                                                                                                                                                          | Combined with the following arylamide of 2,3-hydroxynaphthoic acid                                                                                                                                                                                    | Shade of the dyeing                                                                                               |
|----------------------|----------------------------------------------------------------------------------------------------------------------------------------------------------------------------------------------------------------------------------------------------------------------------------------------------------------------------------------------------------------------------------------------------------|-------------------------------------------------------------------------------------------------------------------------------------------------------------------------------------------------------------------------------------------------------|-------------------------------------------------------------------------------------------------------------------|
| 10                   | (1) 4-amino-1,8-naphthalimide<br>(2) 4-amino-1,8-naphthal-ethylimide<br>(3) 4-amino-1,8-naphthal-ethylimide<br>(4) 4-amino-1,8-naphthal-ethylimide<br>(5) 4-amino-1,8-naphthalphenylimide<br>(6) 4-amino-1,8-naphthal-para-tolylimide<br>(7) 4-amino-1,8-naphthal-meta-tolylimide<br>(8) 4-amino-1,8-naphthal-meta-metadimethyl-phenylimide<br>(9) 4-amino-1,8-naphthal-ortho-ortho-dimethyl-phenylimide | 2'-methoxy-1'-anilide<br>2'5'-dimethoxy-1'-anilide<br>2'-methoxy-1'-anilide<br>4'-methoxy-1'-anilide<br>2'5'-dimethoxy-1'-anilide<br>2'5'-dimethoxy-1'-anilide<br>2'5'-dimethoxy-1'-anilide<br>2'5'-dimethoxy-1'-anilide<br>2'5'-dimethoxy-1'-anilide | Bordeaux<br>Bluish-Bordeaux<br>Bordeaux<br>Bordeaux<br>Violet<br>Bluish-Bordeaux<br>Bordeaux<br>Reddish-violet 70 |
| 15                   | (10) 4-amino-1,8-naphthal-ortho-ortho-dimethyl-phenylimide<br>(11) 4-amino-1,8-naphthal-ortho-ortho-dimethyl-phenylimide<br>(12) 4-amino-1,8-naphthal-ortho-chlorophenylimide<br>(13) 4-amino-1,8-naphthal-ortho-chlorophenylimide<br>(14) 4-amino-1,8-naphthal-ortho-chlorophenylimide                                                                                                                  | 2'-methoxy-1'-anilide<br>4'-methoxy-1'-anilide<br>2'5'-dimethoxy-1'-anilide<br>4'-methoxy-1'-anilide<br>2'-methoxy-1'-anilide                                                                                                                         | Bordeaux<br>Bordeaux<br>Bordeaux<br>Bordeaux<br>Reddish-Violet 80                                                 |
| 20                   |                                                                                                                                                                                                                                                                                                                                                                                                          |                                                                                                                                                                                                                                                       | Bordeaux                                                                                                          |

We claim:

1. As new products, azo dyestuffs of the following formula:

25



30

following formula:

85



90

35

wherein X stands for hydrogen, alkyl, aryl or aralkyl and wherein the aryl residue may be substituted or not, but must contain no free sulfonic or carboxylic group, being claret, garnet or violet dyestuffs of good fastness to washing and chlorine and good to excellent fastness to light.

100

40

3. As new products, azo dyestuffs of the following formula:

105

45



50



110

55

60 wherein X has the same meaning as in the preceding formula, being claret, garnet, vio-

wherein X stands for hydrogen or alkyl and wherein the aryl residue may be substituted

120

or not, but must contain no free sulfonic or carboxylic group, being claret, garnet or violet dyestuffs of a good fastness to washing and chlorine and good to excellent fastness to light.

5. As new products, azo dyestuffs of the following formula:



wherein the aryl residue may be substituted or not, but must contain no free sulfonic or carboxylic group, being claret, garnet or violet dyestuffs of a good fastness to washing and chlorine and good to excellent fastness to light.

5. As new products, azo dyestuffs of the following formula:



45

wherein X stands for hydrogen, alkyl, aryl or aralkyl and Y stands for hydrogen or  $-\text{OCH}_3$ , being violet, garnet, and claret shades of good fastness to washing and chlorine and good to excellent fastness to light.

50

6. As new products, azo dyestuffs of the following formula:



wherein X stands for hydrogen or alkyl and Y stands for hydrogen or  $-\text{OCH}_3$ , being bluish claret, violet or garnet dyestuffs of good fastness, especially good to excellent fastness to light.

7. As new products, azo dyestuffs of the following formula:



wherein Y stands for hydrogen or  $-\text{OCH}_3$ , being bluish claret, garnet or violet shades of good fastness to washing and chlorine and good to excellent fastness to light.

8. As new products, azo dyestuffs of the following formula:



wherein X stands for hydrogen, alkyl, aryl or aralkyl, being garnet and bluish claret shades of good fastness to washing and chlorine and very good to excellent fastness to light.

9. As new products, azo dyestuffs of the following formula:



wherein X stands for hydrogen or alkyl, being garnet and bluish claret shades of good fastness to washing and chlorine and excellent fastness to light.

5 10. As a new product, the azo dyestuff of the following formula:



being water-insoluble and dyeing the material a bluish claret shade of good fastness to washing and chlorine and excellent fastness to light.

11. Material dyed with dyestuffs as claimed in claim 1.
12. Material dyed with dyestuffs as claimed in claim 2.
13. Material dyed with dyestuffs as claimed in claim 3.
14. Material dyed with dyestuffs as claimed in claim 4.
15. Material dyed with dyestuffs as claimed in claim 5.
16. Material dyed with dyestuffs as claimed in claim 6.
17. Material dyed with dyestuffs as claimed in claim 7.
18. Material dyed with dyestuffs as claimed in claim 8.
19. Material dyed with dyestuffs as claimed in claim 9.
20. Material dyed with the dyestuff as claimed in claim 10.

In testimony whereof, we affix our signatures.

WILHELM ECKERT.  
WERNER KIRST.

50

55

60

65